

Jan. 21, 1936.

F. M. CLARK

2,028,589

ELECTRICAL APPARATUS

Filed Dec. 21, 1932



Fig. 1.



Fig. 2.



Fig. 3.



Fig. 4.



Inventor:  
Frank M. Clark,  
by *Charles E. Tuller*  
His Attorney.

## UNITED STATES PATENT OFFICE

2,028,589

## ELECTRICAL APPARATUS

Frank M. Clark, Pittsfield, Mass., assignor to General Electric Company, a corporation of New York

Application December 21, 1932, Serial No. 648,286

4 Claims. (Cl. 220—82)

The present invention relates to encased electrical apparatus, such for example as transformers, X-ray outfits, high tension bushings, and in general devices which are insulated and cooled by liquid dielectric material which is subject during use to chemical change, such as mineral hydrocarbon oil.

Casings for such apparatus sometimes are made partly of transparent glass, in order to permit ascertainment of a condition of the liquid dielectric material, such for example as its level, its fluidity, or the presence or absence in it of sludge. Sludge is a semi-solid material which forms during use. It is deleterious to the dielectric properties of oil and renders it less efficient as a liquid cooling medium.

I have discovered that appreciable damage results to liquid dielectric material which is subject to acid and sludge formation when exposed in such apparatus to the chemical action of light of relatively short wave length. While no sharp critical limit of wave length can be designated, the most deleterious effect appears to be due to light below about 600 millimicrons of wave length. In accordance with my invention this harmful effect is obviated while still giving view to the liquid dielectric material by the use, as a part of the casing, of colored transparent material which is opaque to light of harmful short wave length, preferably an amber glass.

The invention will be more fully explained in the following description taken in connection with the accompanying drawing in which Fig. 1 is a front elevation view of an encased liquid insulated transformer with a high voltage bushing of the oil-filled type; Fig. 2 is an enlarged view of the upper end of the high voltage bushing with parts broken away to indicate the structure more clearly, and Figs. 3, 4, and 5 are graphs indicating the relative effect on oil of clear and amber glass as a container material.

Like reference characters indicate similar parts in Figs. 1 and 2 of the drawing.

The transformer casing 10 shown in Fig. 1 of the drawing is in communication through a pipe 11 with an expansion tank 12 to permit expansion and contraction due to temperature changes of mineral oil or such liquid dielectric material as may be employed in the casing 10. The tank 10, pipe 11 and expansion tank 12 are filled with such liquid to a level 13 in the expansion tank and the space above the liquid is in communication with the outside air through a breather 14. The expansion tank 12 is provided with a transparent liquid level gauge 15

to indicate the level of the liquid inside the tank and casing.

The high voltage bushing 16, as shown in greater detail in Fig. 2, includes a porcelain shell 17 which is filled with insulating oil 18 in which is immersed a conductor 19 connecting the bushing terminal 20 with the transformer in the casing 10. The oil 18 extends up into and partially fills a transparent liquid level gauge 21 to a level 22. The gauge 21 also serves as an expansion chamber to permit expansion and contraction of the oil 18 in the shell 17 due to temperature changes.

Transformers are often used in locations exposed to sunlight, the exposure being sometimes to indirect sunlight but more often being to intense direct sunlight. The casing 10, pipe 11, expansion tank 12 and bushing shell 17 are formed of opaque materials so that the insulating oil in these parts is protected from outside light. However, the liquid level gauges 15 and 21 must be made of transparent material in order that the levels 13 and 22 of the liquid may be visible. Thus, the small volume of oil in these gauges 15 and 21 is necessarily exposed to any direct or indirect light which reaches the gauges.

I have discovered that light having wave lengths greater than about 600 millimicrons does not affect the type of mineral insulating oil in which electrical apparatus is commonly immersed but that light having substantially shorter wave lengths will cause such oil to deteriorate. If this is permitted to happen, the depreciated oil will gradually diffuse and mix with the good oil with which it is in communication in the main casing 10 and in the bushing shell 17.

The effect of the light of the shorter wave lengths is to cause chemical changes in the oil, and acids and sludge are produced. These reduce the dielectric strength of the oil, attack solid material (resins, pitch and the like) used as insulation in the electrical apparatus immersed in the oil and the sludge is deposited on the apparatus so that it is weakened electrically and heat produced during its operation is less efficiently dissipated.

Some of the effects of light passing through ordinary clear glass are made evident by the graphs shown in Figs. 3, 4, and 5. The absence of effect on the oil by light passing through amber glass also is indicated. In Figs. 3 and 4 is indicated the progressive change in color and acidity due to exposure of oil to light passing

- through clear glass. Little darkening is observed for the first couple of weeks. Thereupon an increasing darkening occurs which is a visual telltale of chemical change. After a period of approximately ten weeks the rate of darkening of the oil begins to fall off, no doubt due to its poorer transmissibility of light. As shown by Fig. 4 the development of acids in the oil takes place substantially coincidentally with color change and at nearly the same rate.
- 10 When the light reaching the oil is transmitted by amber glass no appreciable color or acidity change could be noted for the same period of time.
- 15 The formation of sludge under the influence of light is even more marked than the color change and acid formation. As shown in Fig. 5, a rapid increase of potential sludge occurs in the oil. Sludge when first formed in mineral oil tends to be held in suspension or solution, but, 20 of course, accumulates, and eventually becomes precipitated. The sludging produced by exposure to light transmitted by clear glass over a period of about ten weeks (as indicated by the legend 25 Sludge in Fig. 5) and referred to above as "potential sludge" can be made evident by the so-called bomb test. In accordance with it, samples of oil to be tested are subjected in a bomb at a temperature of 140° C. for about 24 hours to oxygen gas at a pressure of about 250 30 pounds to the square inch. Any sludge formed under these conditions is centrifugally separated and observed, and measured. As made evident by Fig. 5 oil subjected under the test conditions 35 only to light transmitted by amber glass showed hardly an appreciable tendency to sludge as shown by the bomb test.
- In order to prevent or reduce these undesirable results, the liquid level gauges 15 and 21 are formed of material, which is opaque to light rays having wave lengths shorter than about 600 40 millimicrons. While amber glass is preferred, red glass or glass of other color cutting off the short wave lengths of light may be employed.
- 45 Harmful light is thus prevented from reaching the oil and light of the visible spectrum having wave lengths substantially longer than 600 millimicrons clearly discloses the level of the oil but does not harm the oil.
- 50 The invention has been explained in connection with a particular application thereof but it will be apparent that other applications and changes may be made without departing from the spirit of the invention and the scope 55 of the appended claims.

For example, parts of the casing of a fluid-cooled electrical device other than a level indicator or gauge may be made of glass having a color adapted to intercept the undesirably actinic short wave lengths. A varnish or other coating of suitable color on a clear glass may be employed within the scope of my invention.

What I claim as new and desire to secure by Letters Patent of the United States, is:

1. In electrical apparatus, a casing, an electrical conductor in said casing, a body of mineral insulating oil in said casing for insulating said conductor, oil level indicating means comprising a portion of said casing, said portion having the capacity to transmit light, said oil being exposed to light passing through said light transmitting portion, and means for substantially restricting transmission of light through said portion to wave lengths in excess of 600 millimicrons to reduce the depreciation of the insulating value of said oil.

2. In electrical apparatus, a casing, an electrical conductor in said casing, a body of mineral insulating oil in said casing for insulating said conductor, an oil level indicating means comprising a portion of said casing having the capacity to transmit light, said oil being exposed to light passing through the said light transmitting portion, and means including an amber glass member for preventing the passage through said portion of wave lengths of light having a depreciating effect on the insulating value of said oil.

3. In electrical apparatus, a casing, an electrical conductor in said casing, a body of mineral oil in said casing for insulating said conductor, an oil-level indicating means comprising a portion of said casing having the capacity to transmit light, said oil being exposed to light passing through said light transmitting portion, and means including a red glass member for preventing the passage through said portion of wave lengths of light having a depreciating effect on the insulating value of said oil.

4. A high tension electrical transformer bushing comprising a casing, an electrical conductor in said casing, a body of mineral oil in said casing for insulating said conductor, a liquid level gauge glass in the wall of said casing, said gauge glass being composed of amber glass whereby wave lengths of light having a depreciating effect on the insulating value of said oil are substantially excluded from said casing.

FRANK M. CLARK.